

2,715,108

## LUBRICATING COMPOSITIONS

Charles E. Francis, Martinez, Calif., assignor to Shell Development Company, Emeryville, Calif., a corporation of Delaware

No Drawing. Application May 6, 1952,  
Serial No. 286,443

16 Claims. (Cl. 252—51.5)

This invention relates to improved lubricating compositions particularly effective as turbine oils.

The essential requirements of a good lubricating turbine oil are that it be resistant to emulsification and oxidation and that it inhibit corrosion or rusting of metal parts exposed thereto. Lubricants which are normally regarded as effective corrosion and rust inhibiting compositions have been observed to be ineffective in this respect when used as turbine oils. The reason for the inability of such lubricating compositions to effectively function as turbine oil lubricants appears to be due to their inability to resist emulsification in the presence of water.

It is an object of this invention to produce an improved rust and corrosion inhibited turbine oil. Still another object of this invention is to produce a turbine oil which is resistant to emulsification in the presence of water. Another object is that it resists oxidation. Other objects of this invention will appear as the description proceeds.

It has now been discovered that excellent emulsion and oxidation resistant and corrosion inhibiting turbine oils can be prepared by addition (to a base oil) of minor amounts, but in controlled proportions, of: (a) an oil-soluble aliphatic polycarboxylic acid and/or an amide or a partial ester of said acid, (b) an oil-soluble phenolic compound or its thio or seleno analogues, and (c) an aromatic carboxylic acid.

(a) *Oil-soluble aliphatic polycarboxylic acid and derivatives thereof*

The oil-soluble aliphatic polycarboxylic acids can be mono or polyalkyl or alkenyl substituted polycarboxylic acids, wherein the alkyl or alkenyl group or groups contain from 3 to 36 and preferably from 8 to 18 carbon atoms. Such acids include oil-soluble C<sub>6</sub> to C<sub>36</sub> and preferably C<sub>8</sub> to C<sub>18</sub> alkyl or alkenyl malonic, succinic, glutaric, adipic, pimelic, sebacic, azelaic, tartaric, citric, maleic, citraconic acids, of which the preferred acids are C<sub>16</sub> alkenyl succinic acid, C<sub>18</sub> alkenyl succinic acid, C<sub>36</sub> alkenyl succinic acid, C<sub>10</sub>—C<sub>18</sub> alkyl tartaric acid, C<sub>10</sub>—C<sub>18</sub> alkyl malonic acid. Partial or full amides and/or the partial esters of these acids can be used, and include alkyl succinic acid monoamide or alkenyl monooleyl succinate, alkyl monoocetyl sebacate, alkyl monobutyl tartrate, mono-isopropyl citrate, mono 2-ethylhexyl citrate, ester of wax phenol and alkenyl succinic acid, ethyl decenyl succinate, decyl isobutetyl succinate, alkenyl succinic acid mono (-dicyclohexyl)amide, C<sub>16</sub> succinic acid mono(2-ethylhexyl)amide, C<sub>18</sub> alkenyl succinic acid monoamide; alkenyl thiosuccinic acid, alkenyl thio tartaric acid, 2-(1-thiotridecyl)succinic acid, 2-(1-thio-decyl)tartaric acid, 2-(1-thio-amyl)citric acid, etc., and mixtures thereof.

(b) *The oil-soluble phenolic compound*

The oil-soluble phenolic compound can be oil-soluble alkyl phenols, naphthols or their thiol and the selenium analogues. The aromatic phenolic compounds can be alkylated by any known suitable means or they may be natural products such as phenols, cresols, etc., obtained

from petroleum hydrocarbons, coaltars and the like. If the phenolic material is to be alkylated, alkenes and their mixtures containing from 4 to 20 carbon atoms in the molecule can be used as the alkylating material. Mixtures of alkenes derived from paraffin waxes by cracking or from higher fatty alcohols by dehydration, are valuable and easily accessible starting materials. More than one alkyl group may be present in the phenol as in the case of compounds made by the di- or tri-alkylation of phenols with alkenes or alkyl halides or alcohols or ethers or of compounds made by monoalkylation of, for example, a cresol, a xylanol, or carvacrol. Other nuclear substituents may be present provided they do not increase substantially the water solubility of the product. Thus 15 halogen, alkoxy, alkylamino, nitro groups may be present in the phenol. Moreover, di- or polyhydric phenols such as catechol, resorcinol, pyrogallol and the dihydroxy naphthalenes may be alkylated to produce water-insoluble and oil-soluble phenols useful for the purpose of this invention. Specific compounds which are represented by the above general formula and which can be used in compositions of this invention are: 2,4-dimethyl-6-tertiary butylphenol, 2,4,6-trimethylphenol, 2,4-dimethyl-6-tertiary octylphenol, 2,6-dibutyl-4-methylphenol, 2,4-diethyl-6-methylphenol, 2-ethyl-4-octylphenol, 1,4-dihydroxy-2-(2-octyl)benzene, 2,4-dimethyl-6-tertiary butyl naphthol, 2,4-diethyl naphthol, 2,4-dimethyl-6-tertiary butyl thiophenol, 2,4-dimethyl-6-tertiary butyl selenophenol, 2-ethyl-4-octyl thiophenol, 2,4-diethyl-6-methyl thionaphthol, 2,4-dimethyl-6-tertiary octyl tellurophenol, C<sub>14</sub> alkylated cardanol, C<sub>14</sub> alkylated thiocardanol, dodecyl phenol, bis-(beta-naphthylamino methyl)-p-tert-amylophenol, o-nitroso m-cresol, p-octyl aminophenol, dibutyl resorcinol, 2,6-di-tertiary butyl-4-methylphenol, 2,4-di-tertiary butyl-6-methylphenol, 2,4-di-sec-butyl-6-tertiary-butylphenol, 2,4-di-n-butyl-6-tertiary-octylphenol, 2,6-di-tertiary-butyl-4-benzylphenol, 2,6-di-tertiary-amyl-4-methylphenol, 2,4-di-tertiary-amyl-6-methylphenol, 2,4,6-tri-tertiary-butylphenol, 2,6-di-tertiary-butyl-4-methylthiophenol, 2,4-di-tertiary-butyl-6-methylthiophenol, 2,4-dimethyl-6-tertiary-butylthiophenol, 2,4-dimethyl-6-tertiary-octylthiophenol, 2,6-di-tertiary-amyl-4-methylthiophenol, 2,4,6-tri-tertiary-amylthiophenol, 2,2'-methylene bis(4-methyl-6-tertiary-butylphenol), 2,2'-methylene bis(4,6-di-tertiary-octylphenol), 2,2'-methylene bis(4-methyl-6-tertiary-amylophenol), 2,2'-methylene bis(4-methyl-6-tertiary-octylphenol), 2,2'-methylene bis(4-methyl-6-tertiary-butylthiophenol), 2,2'-methylene bis(4,6-di-tertiary-butylthiophenol), 2,2'-methylene bis(4,6-di-tertiary-amylophenol), 2,2'-methylene bis(4-methyl-6-tertiary-amylophenol), 2,2'-methylene bis(4-methyl-6-tertiary-octylthiophenol), (2-hydroxy-3-tertiary-butyl-5-methylphenyl)-furylmethane, (2-hydroxy-5-tertiary-butylphenyl)-furylmethane, 1,1-bis(2-hydroxy-3-tertiary-butyl-5-methylphenyl) isobutane, bis(2-hydroxy-3-tertiary-butyl-5-methylphenyl) phenylmethane, 2,2-bis(2-hydroxy-3-tertiary-butyl-5-methylphenyl)propane, 2,2-bis(2-hydroxy-3-tertiary-butyl-5-methylphenyl)butane, and mixtures thereof.

(c) *Aromatic acids*

Aromatic acids which can be used in combination with the above two classes of additives, in order to effect de-

65 mulsification can be represented by the general formula:



wherein Ar is an aromatic nucleus; X' may be a non-polar or polar radical attached to the aryl nucleus; X may 70 be a hydrocarbon radical containing if desired, a polar group; Z is a carboxylic acid group such as CYYH, wherein both Y's are selected independently from oxygen,

sulfur, selenium, and tellurium, said acid group being attached directly to the aryl nucleus or linked to it through X; m may be zero or an integer of from 1 to 3; n may be zero or one and y may be an integer of 1 or 2.

Representative acids are: benzoic, phthalic, toluic, 5 xylid, phenyl fatty acids, e. g., phenyl acetic to phenyl stearic acids, cinnamic acid, salicylic acid, mandelic acid, phenyl glyoxylic acid, benzoyl propionic acid, phenyl laevulinic acid, phenyl alkyl succinic acid, benzyl alkyl succinic acid, phenyl alkyl glutaric acid, o-vinyl benzoic acid, phenyl angelic acid, naphthoic acid, naphthyl stearic acid, anthranilic acid, mercapto (phenyl, tolyl, xylid, xenyl, naphthyl, anthracyl) fatty acids, e. g., phenyl mercapto acetic to phenyl mercapto stearic acid, ethyl mercapto phenyl acetic acid, alkyl mercapto benzene-4-carboxylic acid.

The base for additives of this invention can be an oleaginous material, i. e. any natural or synthetic material, having lubricating properties. Thus the base may be a hydrocarbon oil obtained from a paraffinic, naphthenic, Mid-continent or Coastal stock and/or mixtures thereof and preferably base stocks which have been highly refined. The viscosity of these oils may vary over a wide range such as from 50 SUS at 100° F. to 100 SUS at 210° F. Synthetic oils include olefin polymers, silicone fluids, 25 organic phosphates, esters of polycarboxylic acid, e. g. di-2-ethylhexyl sebacate, adipate and the like. Mixtures of synthetic and natural base oils also can be used.

The additive combination of this invention is used in amounts of about 1% or less and preferably in a total amount of less than 0.9%. The phenolic compound is present in the predominant amount of about 0.5%. The polycarboxylic acid (or derivative thereof) is generally used in amounts of from 0.01 to .2%, while the aromatic acid is present in the additive mixture in the least amount, generally in an amount of about 0.01% or less, based on the finished composition.

The general formula of compositions of this invention can be set forth as follows:

|                                                                   | General Range       | Preferred Range      |
|-------------------------------------------------------------------|---------------------|----------------------|
| Oil-soluble aliphatic polycarboxylic acid and derivatives thereof | Percent<br>0.01-0.2 | Percent<br>0.01-0.05 |
| Oil-soluble phenolic compound                                     | 0.01-1.0            | 0.1-0.8              |
| Aromatic acid                                                     | 0.001-0.01          | 0.001-0.01           |
| Base Oil                                                          | Balance             | Balance              |

Preferred compositions of this invention are illustrated by the following examples:

| Composition A:                        | Per cent by weight |
|---------------------------------------|--------------------|
| C <sub>18</sub> alkenyl succinic acid | 0.025              |
| 2,6-ditert-butyl-4-methyl phenol      | 0.5                |
| Benzoic acid                          | 0.003              |
| Mineral oil                           | Balance            |

| Composition B:                        | Per cent by weight |
|---------------------------------------|--------------------|
| C <sub>18</sub> alkenyl succinic acid | 0.025              |
| 2,6-ditert-butyl-4-methyl phenol      | 0.5                |
| Cinnamic acid                         | 0.003              |
| Mineral oil                           | Balance            |

| Composition C:                        | Per cent by weight |
|---------------------------------------|--------------------|
| C <sub>18</sub> alkenyl succinic acid | 0.025              |
| 2,6-ditert-butyl-4-methyl phenol      | 0.5                |
| Anthranilic acid                      | 0.003              |
| Mineral oil                           | Balance            |

| Composition D:                        | Per cent by weight |
|---------------------------------------|--------------------|
| C <sub>18</sub> alkenyl succinic acid | 0.02               |
| 2,6-ditert-butyl-4-methyl phenol      | 0.5                |
| Salicylic acid                        | 0.003              |
| Mineral oil                           | Balance            |

| Composition E:                                      | Per cent by weight |
|-----------------------------------------------------|--------------------|
| C <sub>10</sub> -C <sub>18</sub> alkyl malonic acid | 0.03               |
| 2,4-diocetyl-6-methyl phenol                        | 0.6                |
| Mandelic acid                                       | 0.003              |
| Mineral oil                                         | Balance            |

| Composition F:                                       | Per cent by weight |
|------------------------------------------------------|--------------------|
| C <sub>10</sub> -C <sub>18</sub> alkyl tartaric acid | 0.04               |
| 2,6-ditert-butyl-4-methyl phenol                     | 0.6                |
| Cinnamic acid                                        | 0.02               |
| Mineral oil                                          | Balance            |

| Composition G:                                          | Per cent by weight |
|---------------------------------------------------------|--------------------|
| C <sub>36</sub> alkenyl succinic acid                   | 0.03               |
| 2,2 - methylene bis(4 - methyl - 6 - tert-butyl phenol) | 0.6                |
| Benzoic acid                                            | 0.02               |
| Mineral oil                                             | Balance            |

| Composition H:                                                       | Per cent by weight |
|----------------------------------------------------------------------|--------------------|
| Monoester of oleyl alcohol and C <sub>18</sub> alkenyl succinic acid | 0.03               |
| 2,6-ditert-butyl-4-methyl phenol                                     | 0.5                |
| Toluic acid                                                          | 0.01               |
| Mineral oil                                                          | Balance            |

| Composition I:                                  | Per cent by weight |
|-------------------------------------------------|--------------------|
| C <sub>18</sub> alkenyl succinic acid monoamide | 0.04               |
| 2,4,6-tritert-amyl phenol                       | 0.6                |
| Benzoic acid                                    | 0.01               |
| Mineral oil                                     | Balance            |

In order to illustrate the effectiveness of compositions in resisting emulsification and in inhibiting corrosion and rust, the following compositions were formulated and tested by the "Navy Emulsion Test," Method 320.1 of Federal Specification VV-L-791; the Salt Water Rust test (ASTM D-665-50T) and the Turbine Oil Stability test (ASTM D-943-47T).

| Composition                | I<br>Navy Emulsion Test <sup>1</sup><br>(F. S. 320.1<br>VV-L-791) | II<br>Rust Test <sup>2</sup><br>(ASTM<br>D-665-50T) | III<br>Turbine Oil <sup>3</sup><br>Stability Test<br>(ASTM<br>D-943-47T) |
|----------------------------|-------------------------------------------------------------------|-----------------------------------------------------|--------------------------------------------------------------------------|
| Composition A              | Excellent                                                         | Excellent                                           | Excellent                                                                |
| Composition B              | do                                                                | do                                                  |                                                                          |
| Composition C              | do                                                                | do                                                  |                                                                          |
| Composition D              | do                                                                | do                                                  |                                                                          |
| Composition X <sup>a</sup> | Poor                                                              |                                                     |                                                                          |
| Composition Y <sup>b</sup> | do                                                                |                                                     | Poor                                                                     |
| Composition Z <sup>c</sup> |                                                                   | Poor                                                |                                                                          |

<sup>1</sup> Excellent—complete demulsification in less than 15-30 minutes in both distilled and synthetic sea water.

<sup>2</sup> Fair—at least 1-3 ml. of emulsion remains around 30 minutes.

<sup>3</sup> Poor—at least 5-80 ml. of emulsion remains after 30 minutes.

<sup>2</sup> Excellent—no rust after 48 hours.

Fair—some rust noted after 48 hours.

Poor—rust noted in less than 24 hours.

<sup>3</sup> Excellent—over 1,000 hours.

Fair—less than 600 hours.

Poor—less than 200 hours.

<sup>a</sup> Composition X comprises mineral oil base having incorporated therein about 0.3% each of C<sub>18</sub> alkenyl succinic acid and 2,6-ditert-butyl-4-methyl phenol.

<sup>b</sup> Composition Y comprises mineral oil base having incorporated therein about 0.3% C<sub>18</sub> alkenyl succinic acid.

<sup>c</sup> Composition Z comprises mineral oil base having incorporated therein about 1% of 2,6-ditert-butyl-4-methyl phenol.

As can be noted from the above test results, compositions of this invention are excellent rust inhibitors and are resistant to emulsification.

Other additives can be added to compositions of this invention such as oiliness agents, extreme pressure agents, anticlogging agents and the like, in amounts of from 0.001% to 5% by weight.

In addition to being excellent turbine oils, compositions of this invention can be utilized as hydraulic oils, cutting fluids, drawing and rolling oils and the like.

I claim as my invention:

1. An improved lubricant consisting essentially of a major amount of a mineral lubricating oil and minor amounts, sufficient to inhibit oxidation and corrosion of (a) an oil-soluble organic compound selected from the group consisting of oil-soluble hydrocarbyl-substituted

aliphatic polycarboxylic acids, their monoesters and monoamides, (b) an oil-soluble phenolic compound, and a minor amount of about 0.01%, which amount is sufficient to effect complete demulsification, of (c) organic acidic compound selected from the group consisting of benzoic acid, salicylic acid, anthranilic acid, cinnamic acid and toluic acid.

2. An improved lubricant consisting essentially of a major amount of a mineral lubricating oil and minor amounts, sufficient to inhibit oxidation and corrosion of (a) an oil-soluble hydrocarbyl substituted aliphatic dicarboxylic acid, (b) an oil-soluble alkyl phenol, and a minor amount of about 0.01%, which amount is sufficient to effect complete demulsification, of (c) organic acidic compound selected from the group consisting of benzoic acid, salicylic acid, anthranilic acid, cinnamic acid and toluic acid.

3. An improved turbine oil consisting essentially of a major amount of a mineral lubricant oil and minor amounts, sufficient to inhibit oxidation and corrosion of (a) an oil-soluble alkenyl substituted aliphatic dicarboxylic acid, (b) an oil-soluble polyalkyl phenol, and a minor amount of about 0.01%, which amount is sufficient to effect complete demulsification, of (c) organic acidic compound selected from the group consisting of benzoic acid, salicylic acid, anthranilic acid, cinnamic acid and toluic acid.

4. An improved turbine oil consisting essentially of a major amount of a mineral oil and minor amounts, sufficient to inhibit oxidation and corrosion of (a) an oil-soluble  $C_{18}$  alkenyl succinic acid, (b) an oil-soluble trialkyl phenol and a minor amount of about 0.01%, which amount is sufficient to effect complete demulsification, of (c) organic acidic compound selected from the group consisting of benzoic acid, salicylic acid, anthranilic acid, cinnamic acid and toluic acid.

5. An improved turbine oil consisting essentially of a major amount of a mineral oil and minor amounts, sufficient to inhibit oxidation and corrosion of (a) an oil-soluble  $C_{18}$  alkenyl succinic acid, (b) an oil-soluble 2,6-ditert-butyl-4-methyl phenol, and a minor amount of about 0.01%, which amount is sufficient to effect complete demulsification, of (c) a benzoic acid.

6. An improved turbine oil consisting essentially of a major amount of a mineral oil and minor amounts, sufficient to inhibit oxidation and corrosion of (a) an oil-soluble  $C_{18}$  alkenyl succinic acid, (b) an oil-soluble 2,6-ditert-butyl-4-methyl phenol, and a minor amount of about 0.01%, which amount is sufficient to effect complete demulsification, of (c) a cinnamic acid.

7. An improved turbine oil consisting essentially of a major amount of a mineral oil and minor amounts, sufficient to inhibit oxidation and corrosion of (a) an oil-soluble  $C_{18}$  alkenyl succinic acid, (b) an oil-soluble 2,6-ditert-butyl-4-methyl phenol, and a minor amount of about 0.01%, which amount is sufficient to effect complete demulsification, of (c) an anthranilic acid.

8. An improved turbine oil consisting essentially of a major amount of a mineral oil and minor amounts, sufficient to inhibit oxidation and corrosion of (a) an oil-soluble  $C_{18}$  alkenyl succinic acid monoamide, (b) an oil-soluble trialkyl phenol, and a minor amount of about 0.01%, which amount is sufficient to effect complete demulsification, of (c) an aromatic monocarboxylic acid.

9. An improved turbine oil consisting essentially of a major amount of a mineral oil and minor amounts, sufficient to inhibit oxidation and corrosion of (a) an oil-soluble  $C_{18}$  alkenyl succinic acid, (b) an oil-soluble 2,2'methylene bis(4-methyl-6-tert-butyl phenol), and a minor amount of about 0.01%, which amount is sufficient to effect complete demulsification, of (c) benzoic acid.

10. A turbine oil capable of resisting emulsification having the following formula:

|                                  | Per cent |
|----------------------------------|----------|
| $C_{18}$ alkenyl succinic acid   | 0.025    |
| 2,6-ditert-butyl-4-methyl phenol | 0.5      |
| Benzoic acid                     | 0.003    |
| Mineral oil                      | Balance  |

11. A turbine oil capable of resisting emulsification having the following formula:

|                                  | Per cent |
|----------------------------------|----------|
| $C_{18}$ alkenyl succinic acid   | 0.025    |
| 2,6-ditert-butyl-4-methyl phenol | 0.5      |
| Cinnamic acid                    | 0.003    |
| Mineral oil                      | Balance  |

12. A turbine oil capable of resisting emulsification having the following formula:

|                                  | Per cent |
|----------------------------------|----------|
| $C_{18}$ alkenyl succinic acid   | 0.025    |
| 2,6-ditert-butyl-4-methyl phenol | 0.5      |
| Anthranilic acid                 | 0.003    |
| Mineral oil                      | Balance  |

13. A turbine oil capable of resisting emulsification having the following formula:

|                                  | Per cent   |
|----------------------------------|------------|
| $C_{18}$ alkenyl succinic acid   | 0.1-0.8    |
| 2,6-ditert-butyl-4-methyl phenol | 0.01-0.05  |
| Benzoic acid                     | 0.001-0.01 |
| Mineral oil                      | Balance    |

14. A turbine oil capable of resisting emulsification having the following formula:

|                                  | Per cent   |
|----------------------------------|------------|
| $C_{18}$ alkenyl succinic acid   | 0.1-0.8    |
| 2,6-ditert-butyl-4-methyl phenol | 0.01-0.05  |
| Cinnamic acid                    | 0.001-0.01 |
| Mineral oil                      | Balance    |

15. A turbine oil capable of resisting emulsification having the following formula:

|                                  | Per cent   |
|----------------------------------|------------|
| $C_{18}$ alkenyl succinic acid   | 0.1-0.8    |
| 2,6-ditert-butyl-4-methyl phenol | 0.01-0.05  |
| Anthranilic acid                 | 0.001-0.01 |
| Mineral oil                      | Balance    |

16. A turbine oil capable of resisting emulsification and oxidation having the following formula:

|                                                                                                                                                     | Per cent    |
|-----------------------------------------------------------------------------------------------------------------------------------------------------|-------------|
| Oil-soluble aliphatic polycarboxylic acid                                                                                                           | 0.01-0.2    |
| Oil-soluble phenolic compound                                                                                                                       | 0.01-1      |
| An aromatic monocarboxylic acid selected from the group consisting of benzoic acid, salicylic acid, anthranilic acid, cinnamic acid and toluic acid | 0.0001-0.01 |
| Mineral oil                                                                                                                                         | Balance     |

#### References Cited in the file of this patent

#### UNITED STATES PATENTS

|           |           |               |
|-----------|-----------|---------------|
| 2,249,333 | Smith     | July 15, 1941 |
| 2,334,158 | Fuchs     | Nov. 9, 1943  |
| 2,340,920 | Archibald | Feb. 8, 1944  |
| 2,434,978 | Zisman    | Jan. 27, 1948 |
| 2,440,530 | Yates     | Apr. 27, 1948 |
| 2,442,672 | Fuchs     | June 1, 1948  |
| 2,459,717 | Perry     | Jan. 18, 1949 |

#### OTHER REFERENCES

70 Performance of Lubricating Oils, by Zuidema Reinhold Pub. Co., New York, 1952, page 130. (Copy in Scientific Library.)